

Patented Oct. 25, 1927.

1,647,096

# UNITED STATES PATENT OFFICE.

CHARLES B. JACOBS, OF WILMINGTON, DELAWARE, ASSIGNOR TO E. I. DU PONT DE NEMOURS & COMPANY, OF WILMINGTON, DELAWARE, A CORPORATION OF DELAWARE.

## EROSIVE RESISTANT FERROUS ALLOY.

No Drawing.

Application filed January 11, 1923. Serial No. 612,016.

This invention relates to a ferrous alloy, and more particularly to an alloy which may be considered as a cast iron of a peculiarly desirable and new character, it having the desirable characteristics of cast iron, such as ability to be simply and inexpensively made and readily cast, but in addition being characterized by extreme hardness, fineness of grain, and great strength. It is 10 the general object of the invention to provide an alloy of the desirable character indicated.

I have found that the addition of relatively high percentages of manganese as 15 compared to those generally present in cast iron gives a variety of iron castings having the properties indicated above. Based on this discovery, the new alloy contains iron, carbon in an amount characteristic of cast 20 iron (in excess of 2%) and manganese in an amount between 3 and 15%, preferably between 9 and 10%. It is readily produced in a cupola according to the procedure generally used in making cast iron.

25 The new alloy is, as stated, extremely hard and fine-grained and, in addition to being hard like chilled iron, is stronger than either chilled iron or grey cast iron, it having a modulus of rupture of from 40,000 to 30,000 pounds per square inch, depending on its content of manganese, the modulus increasing with the manganese content (but 5% of manganese being about the maximum). Its extreme toughness and tenacity 35 is shown by the fact that test bars containing even as high as 10.5% manganese took a permanent set under transverse stress before breaking. Under the same character of stress ordinary cast iron or chilled cast 40 iron breaks with a sharp break. The property of great hardness, combined with toughness, makes the alloy particularly suitable for use in the construction of wearing parts such as liner plates, plows, rabbble 45 blades, crushing rolls, stamp shoes, grinding plates for attrition mills and pulverizers, and in general makes it suitable for a large variety of uses where great hardness, combined with toughness and tenacity, is essential 50 to the life and efficiency of the wearing parts.

The total carbon content of the alloy is greater than 2%, most of the carbon being in the combined form. As indicated, considerable variation in the percentage of

manganese is permissible, variations in the percentage producing various degrees of strength and of resistance to erosion; and it is possible to so design and control the composition of this alloy, or new variety of cast iron, as to make the alloy particularly suitable for particular purposes. Typical examples of the effect of varying the manganese content, other elements remaining the same, are shown in the following 60 65 table:—

| Number. | %Manganese. | Transverse strength (modulus of rupture lbs. per sq. in.). | Remarks.                                                 | 70 |
|---------|-------------|------------------------------------------------------------|----------------------------------------------------------|----|
| 1.....  | 4.35        | 50,000                                                     | Can be drilled or machined with some difficulty.         | 75 |
| 2.....  | 7.67        | 45,900                                                     | Can be drilled or machined only with special hard tools. |    |
| 3.....  | 10.51       | 41,000                                                     | Cannot be drilled or machined.                           |    |

All of the above mixtures make very close grained castings, considerably harder and tougher than ordinary grey iron, which usually show a modulus of rupture of from 33,000 to 39,000# with little or no deflection. The high manganese irons have considerable deflection.

The preferable procedure for making alloys of the present invention is to add to a regular cupola mixture, such for example as used in making an ordinary grey cast iron, a quantity of ferro-manganese, or pure manganese, sufficient to produce in the cast metal 80 the desired manganese content, and to operate the cupola, and cast, in the usual manner. No special precautions in the operation of the cupola or in the molding are required. The function of the manganese in the cupola 85 operation is to convert the greater portion of the graphitic carbon of the iron into a combined carbon in the form of a double carbide of iron and manganese  $(\text{MnFe})_3\text{C}$ . This double carbide is extremely hard and its 90 uniform distribution as such throughout the casting, dissolved in a matrix of iron, hardens and toughens the whole structure of the casting.

Various additions of other elements to the 100 alloy, for example to give special properties and characteristics especially adapting the alloy to particular uses, may be made without sacrifice of the desirable physical properties characterising the alloy in general, I having 110

found that considerable latitude in making up the cupola charges is permissible. For example, chromium in quantities of from, say, 1 to 5% (the percentage of iron being correspondingly reduced) may be added to the alloy with advantage since it particularly well adapts the alloy for castings destined to be subjected in use to high temperatures, such as rabble blades and plows for ore roasting 5 furnaces where the temperature is high and where the parts are subjected to oxidation as well as erosion. While high manganese iron is itself considerably more resistant to oxidation at temperatures ranging from 10 1500 to 1800° F. than is ordinary cast iron or steel, its resistance can be increased by the addition of chromium as indicated. Again, steel scrap or special grades of pig iron, with high or low silicon may be added to the cupola 15 mixture.

Since the addition of manganese to cast iron eliminates sulphur to a large extent, the sulphur content of the alloy is extremely low. This too tends to strengthen and 20 toughen the iron, especially under elevated temperatures, since high sulphur irons are weak, especially at elevated temperatures.

Merely for the purpose of illustration and comparison I may note that two alloys I 30 have made, typical of the present invention, gave the following analysis (percent) (a) manganese 10.17, combined carbon 2.41, graphitic carbon 1.20, (b) manganese 9.08, combined carbon 2.11, graphitic carbon 1.77, the remainder being of course iron in both 35 cases except for such impurities and so forth, negligible for present purposes, as may have been present. As compared to these, a typical grey iron contained, combined carbon 0.23, graphitic carbon 3.08, and a typical pig 40 iron contained, combined carbon .39, graphitic carbon 2.88 (this, as a matter of fact, being the pig iron used in producing alloy ("b").

As will be understood by those skilled in 45 the art, the carbon content of cast iron varies

in different types and therefore, the carbon content of the present alloy may correspondingly vary. It suffices that such content fall substantially within the limits for cast 50 iron, the invention having to do with an alloy with a cast iron base, and relating to the production of a cast iron of certain characteristics. Therefore, mention of carbon content in the claims is primarily for the 55 purpose of indicating a cast iron alloy. (As commonly understood of course "cast iron" has a carbon content in excess of 2% (say about 2.3% and ranging up to about 4.5%).

I claim:

1. An alloy, having major characteristics of cast iron, and containing manganese in amount giving the alloy a modulus of rupture substantially between 40,000 to 50,000 pounds per square inch.

2. An alloy, having major characteristics of cast iron, comprising 3 to 15% of manganese, in excess of 2% of carbon, and iron.

3. An alloy, having major characteristics of cast iron, comprising 3 to 15% of manganese, in excess of 2% of carbon and the remainder iron.

4. An alloy, having major characteristics of cast iron, comprising about 9 to 10% of manganese, in excess of 2% of carbon, and the remainder iron.

5. An alloy, having major characteristics of cast iron, comprising iron primarily, manganese, and carbon in amount characteristic of cast iron, the manganese being sufficient in amount to give the alloy a modulus of rupture substantially between 40,000 to 50,000 pounds per square inch.

6. An alloy, comprising 3 to 15% of manganese, in excess of 2% of carbon, 1 to 5% of chromium, and the remainder iron.

7. A ferrous alloy containing manganese from about 13 per cent to 15 per cent, carbon from about 3½ per cent to 4½ per cent, and the balance preponderantly iron.

In testimony whereof I affix my signature.  
CHARLES B. JACOBS.